

2,877,103

## ARTIFICIAL ABRASIVE ARTICLES

Richard O. Lane, Munith, Mich., assignor to M & M Research and Development Company, Jackson, Mich., a corporation of Michigan

No Drawing. Application December 7, 1954  
Serial No. 473,762

4 Claims. (Cl. 51—298)

The present invention relates to improvements in abrasive articles and the manufacture thereof, being a continuation-in-part of copending application Serial No. 314,072, filed October 10, 1952.

It has heretofore been proposed, as disclosed in the Hartman Patent No. 1,830,757, granted November 10, 1931, to employ an additive material in the manufacture of abrasive articles to produce an abrasive wheel or the like having self dressing characteristics to control "glazing." The additive material contemplated by Hartman was not comparable to the abrasive grain forming the body of the articles in any physical respects. According to Hartman's disclosure the additive functioned to provide voids by being more friable than the abrasive grains and by being of a less hardness yet capable of being broken out of the molded mass of abrasive grains to leave an irregular face. Thus, the self-dressing was effected by the bodily displacement of the additive to leave a void.

In contrast to the disclosure of the aforesaid Hartman patent, the present invention contemplates an additive material in the form of abrasive grains which are comparable in physical respects to the abrasive grains of the mother matrix. In the form of loosely or weakly bonded abrasive grains dispersed within the mother matrix, the additive, according to the present invention, is bodily dislodged by the action of the work piece presented to the working face of the abrasive article; the present theory being that the self-dressing results from the mechanical fracturing action of the additive upon the abrasive grains of the mother matrix taking place between the work piece and the working face of the abrasive article.

In practicing the present invention, only the form and manner of association of the additive in the mother matrix distinguishes the manufacture of abrasive articles made according to the invention over standard practices in the abrasive art. This holds true without regard to the form of bond of the mother matrix such as vitrified, resinoid, shellac, rubber, silicate, magnesium, oxychloride and metallic.

Being mechanical in nature, the action of the loosely or weakly bonded abrasive additive upon the firmly bonded abrasive body is relatively independent of the type of bonding so long as the bonding and/or processing of the firmly bonded abrasive body does not destroy the functional characteristics of the dispersed loosely or weakly bonded abrasive additive.

Thus, an object of the invention is to provide an improved abrasive article having self-dressing characteristics in use in which a dispersed additive is present in the form of loosely or weakly bonded abrasive grains comparable in physical respects to the firmly bonded abrasive grains of the main body of the abrasive article.

Another object of the invention is to provide an improved abrasive article of the type described in the preceding paragraph in which the additive is in the form of pellets of loosely or weakly bonded abrasive grains dispersed in the firmly bonded matrix of the abrasive article

and the grains of which are readily and bodily dislodged during use of the abrasive article to function as a freed fracturing agent of the firmly bonded abrasive grains of the matrix at the point of contact between the work piece and the abrasive article.

Another object is to provide, as a new article of manufacture, an improved additive for grinding wheels and the like to provide the same with self-dressing characteristics, in the form of pellets or loosely or weakly bonded grains comparable in physical respects to the abrasive grains making up the firmly bonded matrix.

These and other objects and advantages of the present invention will more fully appear from the following specification and appended claims.

In carrying out the present invention the additive for abrasive articles preferably comprises abrasive grains which are comparable in hardness and resistance to fracture to the abrasive grains of the firmly bonded body which make up and provide the structural mass of the abrasive article.

As it is the practice, for example, in the manufacture of grinding wheels to make wheels of many sizes of abrasive grains, it would not be practical to match the grain size of the additive with the grain size of each wheel in which the additive is used. It has been found in practice that it is not necessary to closely match the size of the abrasive grain of the additive with the abrasive grain of the firmly bonded matrix of the wheel in order to obtain good results. For example, with the additive having an abrasive grain size of 80, good results are obtained when the additive is used in grinding wheels having abrasive grain sizes ranging from 16 to 120. Likewise, with a grain size of 150 used in the additive, good results have been obtained from this additive when used in grinding wheels having grain sizes ranging from 150 to 500.

The additive is preferably molded or shaped into pellets by an extrusion process which is facilitated by having the additive mix somewhat sticky and greasy. A typical additive mix would comprise 11,360 grams of 80 grain size green or black silicon carbide; cornstarch 675 grams; carboxyl methyl cellulose 575 grams; a colloidal type clay such as bentonite 350 grams; glycerin 1000 cc.; and water 3000 cc.

The cornstarch, clay and carboxyl methyl cellulose are first dry blended and then these are added to the water and glycerin to form a sticky mass. To this is slowly added the abrasive grains. Thereafter, the mix is agitated until a suitable consistency for extrusion is obtained. This mix is then introduced into a pug mill and extruded through  $\frac{1}{16}$ " holes and cut to  $\frac{1}{16}$ " length to provide the pellets.

The extruded and cut to length pellets are then dried to remove substantially all moisture and thereafter subjected to a calcining operation to eliminate the volatile materials, leaving a complex magnesium aluminum silicate bond, holding the abrasive grains together with a degree of tenacity which may be characterized as loosely or weakly bonded as compared to the bonding of the abrasive grains in the matrix of the grinding wheel. After calcining the pellets may be screened and graded to provide a uniform product with the pellets ranging roughly in size from  $\frac{1}{8}$ " to  $\frac{3}{16}$ " for use in grinding wheels of a diameter in the range of 4" and over. With smaller diameter wheels the pellet size should be proportionately reduced to permit uniform dispersion of the pellets with the matrix.

It is to be understood that the binding materials for the abrasive grains of the pellets may be numerous. In the example given only the bentonite will be present in the pellets after calcining as a functional residue of any consequence. The other ingredients provide wetting,

70

lubricating and filler roles to enable the pellets to be extruded, cut and handled. Kaolin in general may be used in place of bentonite. Also, the same bonding used in the matrix but in materially lesser proportions may be used in making the pellets. As for example, in making the pellets the bonding material would be reduced to the order of 2% of the abrasive grain as compared to 15% of the abrasive grain going to make up the matrix.

To give a typical example of the use of the additive pellets in the manufacture of grinding wheels, 134 lb. 7 oz. of green or black silicon carbide of 46 size grain is mixed with 1640 cc. of a solution of dry dextrine in water (50% dry dextrine and 50% water, approximate) until all the grain is uniformly "wetted." Thereafter, 37 lb., 12 oz. of  $\frac{1}{8}$ " to  $\frac{3}{16}$ " size pellets (previously calcined and graded) are carefully and uniformly dispersed in the "wetted" abrasive grains which make up the main body of the grinding wheels. This dispersion should be carried out with care to avoid any appreciable crushing or disintegration of the pellets.

The bond for the abrasive grain of the matrix of the grinding wheel in the example being given comprises 16 lb. 13 oz. of the following ingredients in the proportion given:

|                  | Percent |
|------------------|---------|
| Feldspar         | 57.35   |
| Kentucky #5 clay | 17.50   |
| Stoneware clay   | 17.50   |
| Silica           | 7.65    |

With this bond is hand-blended 5 lb. 11 $\frac{1}{2}$  oz. of dry dextrine and the blended bond and dextrine is then added to the mixture of the preceding paragraph and a final mixing takes place to provide a uniform blend with the pellets uniformly dispersed therein. This final mixture is then removed to the press room where 3,221 grams of the final mixture is placed in a steel mold of the proper shape to make a 10.250" by 2.250" by 7.025" wheel. The wheel mold is then placed in a hydraulic press and pressure applied until the prescribed thickness is obtained, namely, 2.250"; the tonnage required to carry out this operation being in the order of 1000 to 2000 per square inch of pressing surface.

Following inspection, the pressed wheel is then placed in a humidity dryer to remove the moisture. After being thoroughly dried the vitrification cycle is then carried out for nine days in a tunnel kiln in a well known manner. Thereafter the wheel is sized to 10" by 2" by 7" and mounted upon a steel backing disc and placed in use.

In the example given above it will be noted that the pellets constitute 20% by weight of the batch of the final mixture. Experimentation to date indicates that the percentage of the pellets used may be varied over a rather wide range without materially effecting the improved performance of the grinding wheels. However, good practice would indicate that the range should be in the order of 15% to 25% for best all around results.

It is to be understood that the bonding material for the 46 size abrasive grain of the example given will firmly bond these grains into the main mother matrix of the resulting grinding wheel in the conventional manner. However, the bonding of the pellets in the matrix will be confined to a boundary or skin bonding with the result that the interior abrasive grains of the pellets will retain their original loosely or weakly bonded state. Thus, the 46 size abrasive grains of the mother matrix will all be firmly bonded together while the 80 size abrasive grains of the pellets will be loosely or weakly bonded in the wheel except for the boundary bonding that takes place between the mother matrix and the exterior grains of the pellets.

In the appended claims the term "pellets" is used to designate the small preformed objects made up of a relatively large number of abrasive grains or crystals

bonded together to provide the additive which is mixed into the batch from which the abrasive article is later molded and cured.

I claim:

1. An abrasive article of the type in which the components thereof are batch mixed, molded into shape and cured to provide the structural form of the article consisting essentially of a main body portion constituting the mother matrix of the article, said main body portion being formed of abrasive grains and bonding material therefor, said abrasive grains being firmly and independently bonded to each other to provide the mother matrix with said abrasive grains being the main abrasive grains of the abrasive article and providing in their bonded state the structural strength and wearing surface of the article, pellets of abrasive grain and bonding material, the abrasive grains of said pellets being of similar hardness and resistance to fracture as said main abrasive grains, said pellets being present in said matrix as a batch mixed dispersed additive, the abrasive grains of said pellets being weakly bonded to each other, the bonding material and the amount thereof used in said pellets weakly retaining the abrasive grains of said pellets in bonded association with each other as compared to the firm bonding of said main abrasive grains to each other in said matrix, said abrasive grains of said pellets being of a size and being present in sufficient number in said pellets to provide exteriorly located as well as interiorly located grains, the exteriorly located grains of said pellets having boundary bonding in said matrix with the interiorly located grains of said pellets being free from bonding with said matrix, said interiorly located grains in said pellets being subject to bodily dislodgment in the working surface of said article when in use more readily than said main abrasive grains in said matrix, the abrasive grains of said matrix and said pellets having a hardness of 9 or higher on the Mohs scale, said pellets being of a size substantially  $\frac{1}{8}$ " to  $\frac{3}{16}$ " in diameter, and said pellets constituting in the order of 15% to 25% by weight of the mixture from which the article is molded.

2. An abrasive article as defined in claim 1 in which the main abrasive grains have a size in the range of 16 to 120 and the size of the abrasive grains of the pellets are substantially 80.

3. An abrasive article as defined in claim 1 in which the main abrasive grains have a size in the range of 150 to 500 and the size of the abrasive grains of the pellets are substantially 150.

4. An abrasive article as defined in claim 1 wherein the interior abrasive grains of the pellets are bonded to each other with a tenacity comparable to that resulting from a reduction in bonding material of 15% to 20% of the bonding material of the matrix to provide the weak bonding of the abrasive grains of the pellets in contrast to the firm bonding of the abrasive grains of the matrix.

#### References Cited in the file of this patent

#### UNITED STATES PATENTS

|           |              |               |
|-----------|--------------|---------------|
| 1,133,739 | Morse        | Mar. 30, 1915 |
| 1,830,757 | Hartman      | Nov. 10, 1931 |
| 2,162,600 | Ball         | June 13, 1939 |
| 2,246,362 | Kehoe et al. | June 17, 1941 |
| 2,334,266 | Houchins     | Nov. 16, 1943 |
| 2,463,679 | Buckey       | Mar. 8, 1949  |

#### FOREIGN PATENTS

|         |         |              |
|---------|---------|--------------|
| 163,179 | Germany | Dec. 7, 1902 |
| 172,813 | Germany | July 3, 1906 |

#### OTHER REFERENCES

Webster's New International Dictionary, 2nd edition, pp. 1715-1716, 1940.